

## UNITED STATES PATENT OFFICE

2,120,217

## ORE FLOTATION

Benjamin R. Harris, Chicago, Ill.

No Drawing. Application December 18, 1937,  
Serial No. 180,639

45 Claims. (Cl. 209—166)

My invention relates to the separation of mineral constituents of ores by flotation and related processes such as agglomeration.

The froth flotation of sulphide ores has reached a fairly high stage of development and is successfully practiced today with the use of various agents, particularly the xanthates. The concentration of the mineral values in the non-sulphide ores is still a major problem so far as flotation is concerned although, in the past few years, some new flotation agents have been developed which are somewhat effective in this field.

My invention involves the utilization of new flotation agents which are highly effective in the froth flotation of both sulphide and non-sulphide ores and permit the production of relatively pure concentrates with a high percentage of recovery of desired mineral values.

My invention is also concerned with modifying the surface characteristics of the ore to permit the separation of constituents thereof by the well-known agglomeration or granulation method, of which the Cattermole and Murex processes are illustrative, wherein the ore particles are selectively oiled and wherein the separation is effected by tabling as, for example, on a Wilfley table.

One object of my invention is, accordingly, the provision of a new class of reagents which are highly effective in flotation and agglomeration processes.

Another object is the provision of improved flotation frothing and foaming agents which will, in general, perform and function in either acid or alkaline media.

A further object is the provision of a flotation process which may be employed in the flotation of non-sulphide ores.

Still another object of my invention is the provision of novel procedures for effectively separating mineral values from gangue materials associated therewith in ores and the like by froth flotation and agglomeration procedures.

Still another object of my invention relates to effectively separating soluble salts from each other by either froth flotation or agglomeration methods.

Other objects and features of the invention will become apparent as the description proceeds.

In froth flotation one constituent of an ore is selectively modified by the reagents added. These reagents may modify the mineral surface by chemical action or adsorption or both or may modify the interfacial relations with the liquid. In most cases, it is the function of flotation reagents to so modify interfacial relationships that

the mineral particles to be floated are water repellent. Another function of flotation reagents is to produce a froth in which the selectively modified mineral will be included.

In agglomeration or granulation methods of separation, which methods I include within the scope of the term "flotation", the selectively modified mineral-liquid interface is wetted with an oleaginous substance to produce or increase water repellency and the water repellent oil particles are then separated by mechanical means such as a conventional ore dressing table. In this type of separation, the frothing element necessary in froth flotation procedures need not be present. I have found, however, that it is sometimes advantageous to separate selectively oiled particles by froth flotation and this may be readily done in most cases by the addition of a frothing agent if the particles are not too large. It will be seen, therefore, that the initial steps in agglomeration and flotation processes are fundamentally the same, namely, the production of a selectively modified interfacial relationship between the minerals and the liquid surrounding them, the only difference being in the particular method employed for effecting the actual separation of the mineral particles whose surfaces have been modified.

In my Patent No. 1,917,250, I have disclosed a class of chemical substances which I have found can be used with satisfaction in the flotation of ores and minerals. The chemical substances disclosed in said patent have been described as being possessed of certain groupings which impart to the resulting molecule emulsifying, frothing, penetrating, and, in general, surface modifying properties whereby they may be used for various purposes. In said patent, I have shown said chemical substances to have particular utility as emulsifying agents and as addition agents in the manufacture of margarine, to which latter product they impart the property of substantial decrease in its spattering behavior when it is heated in an open pan. I refer those skilled in the art not only to my aforementioned patent but also to related Patents Nos. 1,917,251; 1,917,252; 1,917,255; 1,917,256; 1,917,257; 1,917,258; 1,917,259; and 1,917,260, for a more complete discussion of the characteristics of these substances and representative processes for preparing them.

In general, the classes of substances which I have discovered can be effectively employed as flotation agents in accordance with my present invention are characterized by the presence of

both lipophile and hydrophile groups in the same molecule in a state of "balance". The important characteristics which distinguish the compounds which I employ herein are intimately related to the role which the substances play in the present invention. They are all either freely soluble in aqueous media or dispersible therein. Many of them are also rather freely dispersible in oleaginous media due to the dual character of the molecule, namely, the presence therein of both lipophile and hydrophile groups.

It will be understood that I employ the term "hydrophile group" to include groups which possess affinity for water and aqueous media. As examples of such groups may be mentioned the following: hydroxy, sulphate, sulphonate, phosphate, pyrophosphate, tetraphosphate, lower molecular weight sulpho-carboxylic acids such as sulpho-acetates, sulpho-propionates, etc., and 20 quaternary ammonium or other hydrophilic nitrogenous or non-nitrogenous groups.

Contrastingly, the lipophile group is a group having a definite affinity for oils and fats and comprises, for example, either an alkyl, aralkyl, 25 aryl, ether or ester group. The lipophile group possesses predominantly hydrocarbon characteristics and, in general, is derived from fats, oils, waxes, mineral oils, other hydrocarbons and the like.

30 The lipophile group with its marked affinity for oils and fats generally causes the molecule of which it is a part to orientate itself so that the lipophile group is in relatively closer proximity to the oil medium or phase as contrasted with the aqueous medium in oleaginous-aqueous emulsions.

For my present purposes, namely, for ore separation treatments, the chemical substances which I employ must possess sufficient lipophile 40 mass and quality in order properly to offset and "balance" the hydrophile group. An excess of either lipophile characteristics or hydrophile characteristics is undesirable because the substance then tends to become either predominantly lipophilic or predominantly hydrophilic 45 and in neither case will the most satisfactory results attend the use thereof in ore separation processes. The so-called "balance" of the two groups, namely, the lipophile and the hydrophile groups, in the molecule may be determined empirically by means of a margarine frying test as 50 described in my prior Patent No. 1,917,250. However, in most cases, those skilled in the art will be able to select substances coming within the 55 class suitable for my present purposes from merely an inspection of the molecule of the compound itself.

In general, the lipophile or non-polar group of my compounds should contain at least eight carbon atoms, although, in some specific cases, compounds having as low as four carbon atoms in the lipophile group are of utility for special purposes, this being dependent, in part, upon the specific character of the lipophile group present 60 in the molecule, as well as upon the location of the two groups in the molecule. As a general rule, the hydrophile and lipophile groups should preferably be at the ends or extremities of the molecule as, for example, in the case of palmityl 65 sodium sulphate wherein the palmityl group or, in other words, the lipophile group, is present at one end of the molecule and the sulphate or hydrophile group is present at the other end of the molecule.

70 75 Among the compounds the use of which for ore

separation purposes falls within the scope of my invention are organic chemical substances having balanced lipophile and hydrophile groups, the lipophile group containing at least eight carbon atoms and the hydrophile group comprising a radical selected from the class consisting of oxygenated sulphur and oxygenated phosphorus inorganic acid radicals. One sub-class thereof which I have found to be particularly useful for the separation of mineral values from associated 10 gangue material is the higher molecular weight alkyl sulphates and sulphonates such as heptyl sulphate, octyl sulphate, nonyl sulphate, decyl sulphate, dodecyl or lauryl sulphate, myristyl sulphate, cetyl sulphate, oleyl sulphate, ricinoleyl sulphate, linoleyl sulphate, palmitoleyl sulphate, stearyl sulphate, ceryl sulphate, myricyl sulphate, melissyl sulphate, branched chain higher alcohol sulphates including the sulphates of branched chain octyl, decyl, dodecyl, tetradecyl, hexadecyl 20 and octadecyl aliphatic alcohols as, for example, 2-ethyl hexanol-1, 2-n butyl octanol-1, 3-ethyl-hexanol-1, and the like, preferably employed in the form of their alkali metal salts, by which I include not only the sodium and potassium salts 25 but also the ammonium salts. In general, the sulphates of the normal straight-chain saturated and unsaturated primary aliphatic alcohols having between 8 and 18 carbon atoms are most satisfactory. The alcohols from which these sulphates 30 are prepared may be produced in any suitable manner as, for example, by the reduction of the corresponding fatty esters in accordance with the Bouveault-Blanc method or, alternatively, by the reduction or catalytic reduction with hydrogen of natural or hydrogenated animal or vegetable 35 fats and oils in accordance with well known practices. Again, the alcohols may be derived from synthetic processes such as by the oxidation of hydrocarbons or may be prepared by saponification of waxes and the like. Alternatively, they 40 may be prepared by reduction of aldehydes or by the Grignard reaction. Still other methods known in the literature may be employed if thought desirable or expedient. It is likewise apparent that mixtures of the foregoing or other 45 alcohols may be sulphated or sulphonated and employed as flotation or ore-treating agents in accordance with the teachings of my invention as, for example, the mixture of alcohols resulting 50 from the hydrogenation of coconut oil or the free fatty acids of coconut oil. Lauryl alcohol comprises about 60% of the total alcohol mixture, the remaining alcohols running from  $C_8$  to  $C_{18}$ . (See German Patents D 56471 IV/120 of August 55 30, 1928, and D 56488 IV/120 of September 4, 1928, for reduction with hydrogen of oils and fats and free fatty acids to produce alcohols.) Again, mixtures of alcohols such as are present in the 60 so-called sperm-oil alcohols, as well as those present in wool fat, may also be sulphated or sulphonated and employed in ore-treating operations in accordance with my invention. Indeed, these higher molecular weight alcohols are generally, if, indeed, not almost invariably, offered 65 on the market in the form of mixtures of different alcohols. If desired for any specific purpose, special fractions which predominate in a certain particular higher molecular weight alcohol may be utilized or, if so desired, the sulphates 70 or sulphonates may be prepared from a single, substantially pure alcohol.

As I have indicated, I may utilize the sulphonates of the higher molecular weight alcohols as distinguished from the sulphates thereof. In 75

other words, I may employ such compounds as 5 octyl sulphonic acid, decyl sulphonic acid, lauryl sulphonic acid, cetyl sulphonic acid, and, in general, the sulphonic acid derivatives corresponding to the above-mentioned sulphates, preferably in the form of their alkali metal or ammonium salts.

The sulphates and sulphonates described above 10 may be represented by the general formula



wherein R is a radical containing a hydrocarbon 15 chain of at least eight carbon atoms, X is a sulphuric or sulphonate group present on the extremity of the radical represented by R, and Y is the radical of a salt-forming compound. In a more specific aspect of my invention, R may represent the residue of a normal primary alcohol containing at least eight carbon atoms.

20 In a still more specific aspect of this phase of my invention, the sulphates may be represented by the general formula



25 wherein R represents the residue of a normal primary alcohol containing from 8 to 18 carbon atoms, and Y represents the residue of a salt-forming compound such as sodium.

Another sub-class of compounds useful for 30 flotation purposes are those compounds which correspond to the higher alkyl sulphates and sulphonates described above but wherein the hydrophile group comprises oxygenated phosphorus instead of oxygenated sulphur. Among these compounds may be mentioned lauryl phosphate, 35 palmityl phosphate, sodium palmityl phosphate, stearyl phosphate, oleyl phosphate, calcium palmityl phosphate, monocholesteryl dihydrogen orthophosphate, dicholesteryl hydrogen orthophosphate, cetyl dihydrogen orthophosphate, melissyl 40 phosphate, melissyl calcium phosphate, dipalmityl sodium orthophosphate, and the like. As in the case of the sulphates and sulphonates described previously, it is generally preferred to employ the oxygenated phosphorus derivatives in the form 45 of their alkali or ammonium salts.

A further sub-class of compounds, useful for ore separation processes, are compounds having balanced lipophile and hydrophile groups and comprising derivatives of polyhydroxy substances 50 through which are linked lipophile and hydrophile radicals. In general, these compounds are relatively high molecular weight aliphatic or fatty ethers and esters of polyhydroxy substances 55 wherein a hydrophile group, such as an oxygenated inorganic acid radical, is attached to the polyhydroxy nucleus. More specifically, these compounds may take the form of higher fatty acid esters of aliphatic polyhydric alcohols 60 wherein the hydrogen of at least one of the remaining hydroxy groups of the polyhydric alcohol is replaced by a sulphate, a lower molecular weight sulpho-carboxylic acid or a phosphate radical. Among such compounds may be mentioned, 65 by way of illustration, monostearin sodium sulphoacetate, mono-oleic acid ester of diethylene glycol sulphoacetate, monostearic acid ester of diethylene glycol sodium sulpho-acetate, dodecyl diethylene glycol ether sulphate (mono- 70 ethanolamine salt), stearyl diethylene glycol dihydrogen orthophosphate, lauryl diethylene glycol ammonium sulphate, monolauryl sulphoacetate, sulphates of ethers of diethylene glycol with coconut oil mixed fatty alcohols, mixed coconut oil fatty acid mono-esters of diethylene glycol 75

sulphate (neutralized with sodium, potassium, ammonium or the like) mixed coconut oil fatty acid mono-esters or mono-oleic acid ester of glycerol mono-sulphate (neutralized as indicated), sodium salt of the sulphate of diethylene glycol 5 mono-n-butyl ether, ammonium salt of oleyl and stearyl diethylene glycol, sodium salt of mono-n-capryl diethylene glycol sulphate, monoethanolamine salt of the sulphate of diethylene glycol mono-n-butyl ether, mono-olein disulphate, sulphate 10 of the mono-oleic acid ester of diglycerol, sulphates of mono-fatty acid esters of glycerol such as monostearin mono-sulphate, and the like. For an even more complete disclosure of compounds of this type, reference may be had to my 15 Patents No. 2,023,387, issued December 3, 1935 and No. 2,026,785, issued January 7, 1936, and to my copending application, Serial No. 627,096, filed July 30, 1932.

Other compounds having utility for my purposes, and possessing balanced lipophile and hydrophile groups, are the lower molecular weight sulpho-carboxylic acid esters of the higher molecular weight alcohols referred to hereinabove in connection with the description of the higher 25 alkyl sulphates and sulphonates, including, for example, octyl sulphoacetate, decyl sulphoacetate, lauryl sulphoacetate, lauryl sulpho-propionate, myristylsulphoacetate, cetyl sulphoacetate, cholesterol sulphoacetate, oleyl sulphoacetate, stearyl 30 sulphoacetate, ricinoleyl sulphoacetate, linoleyl sulphoacetate,  $\beta$ -ethyl-hexyl sulphoacetate, and the like, preferably in the form of their alkali metal, ammonium, or organic amine, such as ethanolamine, salts.

35 A further subclass of compounds having utility in ore separating treatments, and having balanced lipophile and hydrophile groups, are certain derivatives of polyhydroxy substances or polyhydroxycarboxylic acids including, for example, 40 such compounds as monostearic acid ester of dextrose, mono-stearic acid ester of sucrose, mannitol mono-palmitate, stearyl tartaric acid, mucic acid mono-palmitate, stearyl malic acid, digitonincholesteride, and the like. For a further disclosure 45 of such compounds, reference may be had to my Patent No. 1,917,257, above mentioned, and to my Patent No. 2,025,984, issued December 3, 1935.

Still another group of reagents which I have 50 found effective for my present purposes, and falling within the class of organic chemical substances having balanced lipophile and hydrophile groups with a lipophile group having at least eight carbon atoms, are organic nitrogenous substances. 55 These compounds include organic nitrogen-containing halides having a hydrocarbon group of at least eight and preferably at least twelve carbon atoms and, more specifically, aliphatic derivatives of anion-containing heterocyclic compounds such as aliphatic hydrocarbon derivatives of pyridinium halides such as pyridinium chloride or bromide. Among the specific compounds falling within this class may be mentioned, by way of illustration, cholesteryl 60 ester of betaine hydrochloride, (carbocholesteroxy) methyl trimethylammonium chloride, cholesteryl ester of betaine hydrobromide, palmityl ester of betaine hydrochloride or hydrobromide, (carbopalmitoxy) methyl pyridinium bromide, melissyl ester of betaine hydrobromide, (carbocholesteroxy) methyl pyridinium bromide, (carbocholesteroxy) methyl dimethylphenyl ammonium bromide, (carbocholesteroxy) methyl quinaldinium bromide, cholesteryl dimethyl- 75

aminoacetate hydrobromide, palmityl ester of dimethyl-aminoacetic acid hydrobromide, palmito-glycine, palmito-leucine, stearyl creatinine (sodium salt), stearyl glutamic acid and the like. Additional examples of compounds falling within this sub-class may be found in my Patent No. 2,023,075, issued December 3, 1935.

For the preparation of the higher aliphatic or higher fatty acid esters described hereinabove, such as monostearin sulphate, monolauric acid ester of diethylene glycol, and the like, the term "higher" being employed to mean at least eight carbon atoms, the following acids may be employed as well as mixtures thereof: saturated 15 and unsaturated aliphatic and fatty acids including caprylic, capric, stearic acid, hydroxystearic acid, oleic acid, lauric acid, myristic acid, coconut oil mixed fatty acids, linoleic acid, ricinoleic acid, palmitic acid, melissic acid; and mixed 20 higher fatty acids derived from animal and vegetable oils and fats, whether hydrogenated or not, such as cottonseed oil, corn oil, soya bean oil, sesame oil, fish oils, lard, oleo oil, and others, such as the fatty acids derived from waxes like 25 beeswax and carnauba wax.

I have mentioned hereinabove that the sulphates, sulphonates and other oxygenated sulphur and phosphorus derivatives are preferably employed in the form of their alkali metal or 30 ammonium salts. In certain instances, other cations may be present in place of sodium, potassium or ammonium, as, for example, calcium, magnesium, aluminum, zinc, and organic cationic-functioning or neutralizing compounds such as 35 the aliphatic and aromatic amines including, for example, tertiary amines, pyridine, quinaldine, alkyloamines such as mono-, di- and triethanolamine and mixtures thereof, quaternary ammonium bases such as tetra-methyl and tetra-40 ethyl ammonium hydroxide, and the like.

While flotation reagents may be classified in general into frothers and collectors, this classification is not particularly useful in describing my invention since, under different conditions, 45 these reagents may fall into one or both classifications. In general, reagents of the classes described hereinabove possess frothing properties in at least some degree and, in many cases, certain of these compounds may be used as 50 frothers with the exertion of a minimum of influence on the flotation circuit other than to provide the necessary volume of froth. In other cases, the compounds function simultaneously as frothers and collectors. As an illustration, 55 pounds of the type of lauric acid ester of diethylene glycol ammonium sulphate are highly selective collectors and may be used in conjunction with other agents without interfering with the selective properties thereof. On the other 60 hand, lauric acid ester of diethylene glycol ammonium sulphate and similar compounds function both as frothers and collectors for the separation of such minerals as calcite and apatite from less readily floatable minerals. Again, the 65 higher molecular weight alkyl sulphates are excellent frothing agents and, in many instances, also function as collecting agents.

As previously described, the reagents which I employ herein selectively modify the interface 70 relationship of certain minerals so that they may be oiled and separated by either froth flotation methods or agglomeration and tabling. In some cases of agglomeration procedures, the oiling is not necessary. Where oiling is employed, it may 75 be done simultaneously with the addition of the

selective interface modifying agents or the oiling may be carried on subsequently in a separate step.

Since the reagents which I employ herein possess good emulsifying and dispersing power, 5 they may be advantageously used to prepare emulsions of petroleum oils, kerosene, vegetable and animal oils, normally solid or liquid higher fatty acids, and to prepare dispersions of other lipophilic solids such as metallic soaps and xanthates. These emulsions or suspensions are useful as collecting agents and the like in the flotation and agglomeration of minerals. These emulsions may be prepared by any of the several methods known in the art. For example, the flotation 10 agents of my invention may be admixed with a small amount of water in a mortar and then oil may be gradually added while continuously stirring or mixing until emulsification is initiated. The oil may then be added more quickly until the 15 formation of the emulsion is completed. It will be understood, of course, that the stability of the emulsion will be affected by various factors including the relative proportions of the flotation agent, water, and oil or the like, the specific type 20 of agent and oil or the like, the pH, and the exact method of preparation. In general, the oil-in-water type of emulsions produces superior 25 results.

I shall now describe the manner in which the 30 novel flotation agents may be used in the actual separation of mineral values from ores containing the same by froth flotation as well as by agglomeration methods.

#### Example I

35

In the concentration of tungsten ore containing scheelite, calcite and quartz, the ore was ground to 100 mesh, the grinding being carried out preferably to keep the amount of fines as low as 40 possible. The ore was then acidified to the extent of about 1.0 lb. of sulphuric acid per ton of pulp. 0.25 lb. of oleic acid per ton of ore and 0.25 lb. of lauric acid ester of diethylene glycol ammonium sulphate per ton of ore were added 45 and the pulp subjected to froth flotation. The froth which contained only calcite was first removed. The acidity was then reduced to about 0.4 lb. per ton of pulp by the addition of caustic soda and the flotation was then continued. The 50 concentrate and tailing obtained in this flotation is shown by the following table:

| Product           | Weight per cent of original ore | Assay percent WO <sub>3</sub> | Recovery | 55 |
|-------------------|---------------------------------|-------------------------------|----------|----|
| Concentrate.....  | 3.6                             | 65.2                          | 93.6     |    |
| Tailing.....      | 74.9                            | 0.04                          | 1.2      |    |
| Original ore..... |                                 | 2.50                          | -----    | 60 |

#### Example II

65

In the treatment of a complex lead-zinc-iron sulphide ore from Utah, having the composition—lead 8.8%, zinc 9.7%, iron 28.2%, and the remainder silica and silicates, the ore was ground to pass a 60 mesh screen and was made into a pulp containing 20% solids. The pulp was then conditioned with 2.0 lbs. of sodium carbonate per ton and then subjected to froth flotation 70 using as a reagent an aqueous emulsion containing 1.0% of lauric acid ester of diethylene glycol ammonium sulphate and 2% of corn oil. An amount of this reagent was initially added to give 0.2 lb. of the lauric acid ester of diethylene 75

glycol ammonium sulphate per ton of ore. The mineralized froth which formed immediately was removed as concentrate No. 1. Additional emulsion to double the original amount was then added and after several minutes further mineralized froth formed, this being removed as concentrate No. 2. When no more mineral appeared in the froth, 0.2 lb. of copper sulphate per ton of ore was added and another concentrate removed which was designated as No. 3. The mineral remaining in the machine was removed as tailings. The analysis of the concentrates and tailings is shown in the following table:

FROTH FLOTATION—UTAH COMPLEX ORE  
Head analysis lead 8.8%—zinc 9.7%—iron 28.2%

| 20                   | Analysis percent |      |     | Recovery percent |    |    |
|----------------------|------------------|------|-----|------------------|----|----|
|                      | Pb               | Zn   | Fe  | Pb               | Zn | Fe |
| 1st concentrate..... | 76.2             | 1.9  | 0.5 | 93               | —  | —  |
| 2nd concentrate..... | 1.8              | 60.5 | 1.9 | —                | 89 | —  |
| 3rd concentrate..... | —                | —    | —   | —                | —  | —  |
| 25 Tailing.....      | .03              | .08  | 1.9 | —                | —  | 86 |

It will thus be seen that the lead, zinc, iron and insolubles have been thoroughly separated. The lauric acid ester of diethylene glycol ammonium sulphate employed in this example may be replaced by other compounds of the types disclosed herein and, in particular, by dodecyl sodium sulphate, butyl ether of diethylene glycol sodium sulphate, oleyl or stearyl diethylene glycol ammonium sulphate, monoethanolamine salt of butyl ether of diethylene glycol sulphate, lauryl sodium sulphonate, normal octyl sodium sulphate, heptyl sodium sulphate, mono-olein disulphate, sulphated oleic acid ester of diglycerol, monostearate, and the like. It will, of course, be evident that not all of these compounds necessarily yield as good results as the lauric acid ester of diethylene glycol ammonium sulphate nor are they necessarily as satisfactory when used in as small amounts as the lauric acid ester of diethylene glycol ammonium sulphate. The corn oil employed in the example may be replaced, with substantially the same results, by cottonseed oil, olive oil, palm oil and the like. Sardine oil, menhaden oil and lard oil may also be used although these are not quite so satisfactory as the aforementioned oils. Petroleum oils of various grades give a somewhat lower selectivity than corn oil or cottonseed oil but may be preferred in certain instances because of their lower cost.

### Example III

In another example, involving the separation of ilmenite from a gangue material composed of phosphate, quartz and garnet, the ore analyzed 1.8%  $TiO_2$  as ilmenite. The ore was ground to pass a 60 mesh screen and conditioned with 0.2 lb. sulphuric acid and 0.1 lb. of ferric ammonium sulphate per ton. The pulp, containing 20% solids, was then subjected to froth flotation using an emulsion of 2.0% crude oil in water containing 1% of mixed coconut oil fatty acid mono esters of glycerol sulphate neutralized with triethanolamine, an amount of the emulsion equivalent to 0.5% of oil per ton of ore being employed. The concentrate contained 37% of  $TiO_2$ , representing a recovery of 94.5%.

### Example IV

75 As still another example, malachite was floated

from a New Mexico copper ore using an aqueous emulsion containing 1% sardine oil and 1% normal decyl sodium sulphate. The ore contained 1.0% copper and produced an uncleaned concentrate analyzing 38.2% copper.

The use of emulsions, as described above, was effective in a slightly acid circuit on chromite ores, rutile ores, hematite ores, and magnetite ores. In alkaline circuit, with the addition of copper sulphate, silica, limestone, barite, fluor-spar, and magnesite were floated. In some cases particularly when the minerals were adapted to be freed at relatively coarse sizes, the froth flotation was effectively replaced by agglomeration or granulation and tabling. In this latter instance, the first step of the process, namely, selective oiling, was carried out exactly as in the case of the use of emulsions for froth flotation as described hereinabove.

### Example V

An ore of rutile and apatite, containing 3.6%  $TiO_2$  as rutile, was ground to pass through a 20 mesh screen and conditioned in a thick pulp with an aqueous emulsion containing corn oil and mixed coconut oil mono-fatty acid esters of diethylene glycol ammonium sulphate. Using 0.4 lb. of the sulphated reagent per ton and 3 lbs. of corn oil per ton, the ore was conditioned by thoroughly mixing. Water was then added to produce a pulp suitable for tabling. The results are shown in the following table:

| Product                 | Wt. per cent | $TiO_2$ per cent |
|-------------------------|--------------|------------------|
| Table concentrates..... | 4.1          | 88.0             |
| Table tails.....        | 95.9         | 4.9              |

As a general rule, it is preferable to add the surface modifying agent first in the very thin pulp followed by the addition of the oil and then the subsequent dilution of the pulp to the proper density for separation on the table. As illustrative of such practice, the treatment of an iron ore may be considered.

### Example VI

An ore from the Lake Superior district, containing 30.2% iron, the gangue being silica, was ground to pass through a 14 mesh screen and mixed with a small amount of water, 2.0 lbs. of sulphuric acid and 1.0 lb. of the mixed coconut oil fatty acid mono esters of diethylene glycol ammonium sulphate per ton of ore. Crude mineral oil in the amount of 6 lbs. per ton was then added and the entire mass mixed. The results, after dilution and tabling, were as follows:

| Product                 | Wt. per cent | Fe per cent |
|-------------------------|--------------|-------------|
| Table concentrates..... | 51.2         | 63.2        |
| Table tails.....        | 49.8         | 8.2         |

The process described in Example VI in connection with the concentration of iron ore may be used on chromite, magnetite, apatite, limestone, dolomite, magnesite and bauxite, without special care in the selection of the reagent for the oil. In other cases, however, the selection of the flotation agent is quite critical as, for example, in the separation of sylvite and halite as they occur in Carlsbad, New Mexico. In this latter case, where agglomeration procedures are employed, the flotation agent must be soluble

enough to promote oiling but must selectively affect the interfacial relationship between either the sodium chloride and the potassium chloride and the brine. Since potassium salts are, in general, more insoluble than sodium salts, it is my hypothesis that the flotation agent acts in this case by precipitation of a film of potassium salt, but enough of the flotation agent remains in solution to serve as an oil carrier. An agent which 5 has produced unusually good results for the separation of halite and sylvite is mixed coconut oil fatty acid mono esters of diethylene glycol neutralized with ammonia sodium hydroxide, ethanolamines, such as triethanolamine and the like. Other neutralizing agents may be used but the employment of such agents as indicated above has produced very satisfactory results. The process may be carried out according to several procedures to produce a mixture of brine, mineral 10 oil and the neutralized mixed coconut oil fatty acid mono esters of diethylene glycol sulphate, the oil being selectively adsorbed by the sylvite but not coating the halite, the result being that the sylvite is formed into glomerules of such 15 composition and size that ordinary tabling is sufficient to separate them. The concentrate will consist, in general, of from 85% to 95% potassium chloride, the tailings containing only about 5% or less of potassium chloride. The concentrate 20 may be either dried or otherwise treated to produce a product acceptable for agricultural purposes.

#### Example VII

As an example of the separation of halite and sylvite, an emulsion was formed of 25 lbs. of crude mineral oil, one lb. of neutralized mixed coconut oil fatty acid mono esters of diethylene glycol sulphate and enough brine made from the ore to produce a total of 100 lbs. of emulsion. 35 This emulsion was then added to the ore, which was in the form of a relatively thin pulp of 12 to 16 mesh ore, the proportions being such that about 1½ to 4 lbs. of the sulphate reagent and 40 10 to 15 lbs. of oil were present in about one ton of ore. The ore containing the emulsion was agitated slowly for approximately five minutes until the sylvite agglomerated into particles of sufficient character and size to permit easy separation. The glomerules were easily observed so that it 45 could readily be determined whether or not the product had advanced to a suitable condition for separation on the separating table. Although tabling proved very satisfactory for the separation, any other suitable method of separation 50 commonly used in the ore dressing industries can be substituted therefor.

#### Example VIII

In accordance with another method of separating the sylvite and halite, the crude oil was added to a very thick pulp and the sulphate reagent, previously dispersed in a small amount of water, was introduced into the pulp. By this method, the amount of the sulphate reagent was 60 reduced to 1.6 lbs. per ton of ore. The results of a test made in this way are shown in the following table:

| 70                      | Product | Wt. percent | Percent KCl | Total KCl percent |
|-------------------------|---------|-------------|-------------|-------------------|
| Table concentrates..... | 45.2    | 85.1        | 95.2        |                   |
| Table tails.....        | 54.8    | 4.0         | 4.8         |                   |
| Composite.....          | 100     | 40.6        | 100         |                   |

#### Example IX

In accordance with still another modification, 5 2000 lbs. of sylvinitite, reduced to a size of about 12 to 16 mesh, were moistened with a brine (a saturated brine prepared from the ore was employed). To this were added 4 lbs. of the ethanolamine salt of mixed coconut oil fatty acid mono-esters of diethylene glycol sulphate, thorough stirring being employed to produce a substantially uniform mixture. 15 lbs. of crude oil were then stirred into the mass and uniformly dispersed therein. 10 Approximately 2000 lbs. of the brine were then incorporated and the total constituting about 2 tons was tabled. A high-grade concentrate of sylvite, averaging about 90% KCl, was obtained with only about 5% KCl in the tailings. The tails may be in part recirculated to increase the proportionate yield of KCl. The concentrate 15 may be dried in any suitable manner as for example, in air, and may then be crushed to give an acceptable agricultural potassium chloride product.

The amount of flotation agent and oil employed 25 are not particularly critical so far as separation is concerned, but, in the interest of economy, it is apparent that no more of the reagent should be used than is sufficient to produce satisfactory separation. It is desirable that not more than enough oil to wet the sylvite particles should be 30 employed because the oil has a tendency to separate out on the table or other equipment used for separation and this requires periodic cleaning which can be avoided if the amount of oil is properly gauged.

While many oleaginous constituents may be 35 employed, the best results appear to be obtained if a crude mineral oil, for example, is used. Gulf Coast crude oils, for example, produce particularly good results. It has also been found that 40 if the crude oil is preliminarily treated to remove some of the volatile constituents, the amount of oil employed in the separation treatment can be decreased and, in general, somewhat better results are obtained.

Other flotation agents with which satisfactory 45 results have been obtained in the agglomeration of sylvite are oleic acid ester of diethylene glycol sodium sulphate, mixed coconut oil fatty acid mono-esters of glycol mono-ammonium sulphate, 50 lauryl sulphonic acid, octyl sulphonic acid, decyl sulphonic acid, and the like. It may also be pointed out that, with any of these, the oiled sylvite may be separated by froth flotation instead of agglomeration and tabling by decreasing the amount of oil and adding a suitable frother if necessary.

The unusual ability of many of these reagents to froth in saturated salt solutions makes them 60 very valuable reagents for water-soluble salt separations by froth flotation methods and they may be used successfully, for example, in the separation of boric acid from potassium sulphate, ammonium chloride from sodium nitrate, sylvite from halite, the concentration of potassium sulphate and the separation thereof from its associated halite in the mineral langbeinite, the separation of salts of barium, lead, zirconium, and ferric iron from salts of potassium, zinc, calcium, magnesium and the like, and for other water-soluble 65 salt separations.

In carrying out the separation of soluble salts 70 from each other by froth flotation procedures, it is unnecessary to resort to oiling as described hereinabove. For effecting the separation, for 75

example, of sylvite from halite by froth flotation without oiling, according to my hypothesis an agent should be used for precipitating an insoluble potassium salt with a long chain lipophile group outward so as to make the particles water repellent. For this purpose, the alkali metal or ammonium salts of the fatty alcohol sulphates and sulphonates having from 6 to 14 carbon atoms are of utility. Of unusual utility is 10 normal octyl sodium sulphate.

*Example X*

As illustrative of separating soluble salts from each other by a froth flotation process without 15 oiling, a sylvinite ore was ground to pass a 48 mesh screen and conditioned by the addition of a small amount of an aqueous solution of normal octyl sodium sulphate, amounting to approximately 0.8 lb. of the octyl sulphate per ton of ore. 20 The ore was then made up to a 20% pulp in a saturated brine produced from the sylvinite mineral itself and the mass was then subjected to froth flotation. The results obtained are shown in the following table:

| Product                   | Weight percent | KCl percent | Total KCl percent |
|---------------------------|----------------|-------------|-------------------|
| Cleaner concentrates..... | 42.8           | 95.6        | 94.2              |
| Middlings.....            | 6.8            | 25.2        | 3.2               |
| Rougher concentrates..... | 50.8           | 85.8        | 98.8              |
| Tailings.....             | 49.2           | 1.4         | 1.7               |
| Composite.....            | 100            | 42.9        | 100               |

Since, according to my hypothesis, this flotation action would appear to depend upon the formation of an insoluble potassium salt, the method would be applicable to the separation of any mineral containing a soluble potassium salt. Thus, for example, cement dust containing 10% 35 K<sub>2</sub>O was concentrated by froth flotation by adding 2 lbs. of sulphuric acid per ton and 1.2 lbs. of normal octyl sodium sulphate per ton. The concentrate analyzed 48.7% K<sub>2</sub>O.

I have also found that the flotation of at least 45 many non-sulphide minerals can be inhibited by proper acid concentration. The following table, for example, shows the concentrations at which some of the common minerals are depressed when using a mixture of lauric acid ester of diethylene 50 glycol ammonium sulphate and oleic acid as a froth flotation reagent:

| Mineral            | H <sub>2</sub> SO <sub>4</sub> per ton pulp |
|--------------------|---------------------------------------------|
| Rhodochrosite..... | 4                                           |
| Calcite.....       | 2.0                                         |
| Scheelite.....     | 0.6                                         |
| Apatite.....       | 0.4                                         |
| Hematite.....      | 0.1                                         |

It will be understood that, while the flotation agents of my invention are very valuable in the flotation of non-sulphide minerals, and in this 65 respect represent a distinct advance in the art, they may also be employed for the treatment of various types of sulphide ores. It will likewise be evident that, when substituting other agents than those employed in the specific examples illustrated hereinabove and utilizing the process with different types of ores, it may be necessary to conduct a few simple experiments to determine the most suitable agent for the particular purpose as well as the most satisfactory concentration 70 thereof for the obtention of the best results, it

being, of course, recognized that the treatment of different types of ores and minerals may require certain minor modifications and changes. However, in the light of my disclosures herein, it will be evident to those skilled in the art how to 5 carry out my teachings and produce satisfactory separations.

As previously indicated, the concentration of the flotation agents employed is subject to considerable variation, this being dependent upon the 10 potency of the particular agent selected, the nature of the specific ore treated, the degree or character of the separation desired, and upon other factors which are apparent to those versed in the art. In general, concentrations of about 15 .01% up to several per cent of the agent, based upon the aqueous content of the ore mass being floated, will serve the purpose, the average case generally requiring from about .05% to .7%.

It will be appreciated that I may employ mixtures of the flotation agents described hereinabove in order to obtain novel effects. For example, while dodecyl sodium sulphate is not quite so selective as lauric acid ester of diethylene glycol ammonium sulphate with respect to certain types 25 of ores, mixtures of dodecyl sodium sulphate and lauric acid ester of diethylene glycol ammonium sulphate, with or without oleic acid or other similar collectors, can be used to produce a wide variety of froth textures which can be taken advantage of for the treatment of particular ores.

The novel flotation processes which I have described herein are applicable to the treatment of ores generally. Among the ores which have been treated with very good results in accordance with 35 my invention are tungsten ores, lead-zinc-iron ores, oxidized ores such as lead carbonate, activated blende, kyanite ore, chromite ore, phosphate ores, bauxite, graphite ores, magnetite ores, the separation of silica from various types of ores, 40 mica, zirkite ores, rutile ores, cassiterite ores, iron ores, kaolin, coal, and the like.

It will, of course, be understood, particularly in the light of the examples set forth hereinabove, that the novel froth flotation and agglomeration 45 reagents of the present invention may be employed in conjunction with one or more already known agents such as collecting agents, frothing agents, depressing agents, emulsifying agents, dispersing agents, activating agents, deactivating 50 agents, inhibitors, and, in general, organic and inorganic conditioning agents, and the like. These agents include, among others, mineral and vegetable oils, fuel oil, kerosene, mercaptans, xanthates, organic sulphides, hydrosulphides, carbamates, thiocarbamates, thioureas, di-thiophosphates, azo and diazo compounds, amines such as monoethanolamine, diethanolamines, triethanolamines and pyridine, alkali metal and heavy metal soaps, higher fatty acids such as oleic acid and 55 palmitic acid, sulphonated oils and sulphonated higher fatty acids such as Turkey red oil and sulphonated oleic acid, gelatin, glue, starch, copper sulphate and other salts of copper, mercury and lead, alkali metal sulphides such as sodium sulphide, alkalies such as sodium hydroxide, potassium hydroxide and sodium carbonate, alkali metal silicates such as sodium silicate and other agents which are commonly employed in flotation and agglomeration processes. It will also be understood, as described above, that the flotation 60 circuit may be acid or alkaline depending on the particular ore being separated, the nature of the reagents used and the character of the separations desired.

By controlling the pH of the cir- 75

cuit, selective flotation of various minerals can, in many cases, be very satisfactorily accomplished.

It will be understood that the description of my invention, although, detailed, is to be taken not in a limitative sense but only in a descriptive sense, the scope of my invention being pointed out in the appended claims.

The present application is a continuation-in-part of my prior applications, Serial No. 679,716, filed July 10, 1933 and Serial No. 6,393, filed February 13, 1935.

What I claim as new and desire to protect by Letters Patent of the United States is:

- 15 1. In a process for concentrating non-sulfide minerals by froth flotation, the step of adding to an ore pulp a proportion of an organic chemical substance having balanced lipophile and hydrophile groups, the lipophile group containing at least eight carbon atoms and the hydrophile group comprising a radical selected from the class consisting of oxygenated sulphur and oxygenated phosphorus inorganic acid radicals, and subjecting the pulp to froth flotation.
- 20 2. In a process for concentrating non-sulfide minerals by froth flotation, the step of adding to an ore pulp a proportion of a fatty acid and a proportion of an organic chemical substance having balanced lipophile and hydrophile groups, said lipophile group containing at least eight carbon atoms and the hydrophile group comprising a radical selected from the class consisting of oxygenated sulphur and oxygenated phosphorus inorganic acid radicals, and subjecting the pulp to froth flotation.
- 25 3. In a process for concentrating non-sulfide minerals by froth flotation, the step of adding to an ore pulp an acid in relatively high concentration and a proportion of an organic chemical substance having balanced lipophile and hydrophile groups, the lipophile group containing at least eight carbon atoms and the hydrophile group comprising a radical selected from the class consisting of oxygenated sulphur and oxygenated phosphorus inorganic acid radicals, and subjecting the pulp to froth flotation.
- 30 4. In a process for concentrating non-sulfide minerals by froth flotation, the step of adding to ore pulp an acid, and an organic chemical substance having balanced lipophile and hydrophile groups and having the property of foaming in an acid medium, said lipophile group containing at least eight carbon atoms and the hydrophile group comprising a radical selected from the class consisting of oxygenated sulphur and oxygenated phosphorus inorganic acid radicals.
- 35 5. In a froth flotation process for concentrating non-sulfide minerals, the step of treating a mass of pulp with an acid to produce a concentration equivalent to at least 0.1 lb. of sulfuric acid per ton of pulp and adding an organic substance having lipophile and hydrophile groups in a state of balance in the molecule, the lipophile group having at least eight carbon atoms and the hydrophile group comprising a radical selected from the class consisting of oxygenated sulphur and oxygenated phosphorus inorganic acid radicals.
- 40 6. In a process for concentrating non-sulfide minerals by flotation, the steps of acidifying pulp to the equivalent of at least 0.1 lb. of sulfuric acid per ton, adding oleic acid and an organic chemical substance having balanced lipophile and hydrophile groups, the lipophile group having at least eight carbon atoms and the hydrophile group comprising a radical selected from the class consisting of oxygenated sulphur and oxygenated phosphorus inorganic acid radicals.
- 45 7. In a process for concentrating non-sulfide minerals by flotation, the steps of acidifying pulp to the equivalent of at least 0.1 lb. of sulfuric acid per ton, adding oleic acid and an organic chemical substance having balanced lipophile and hydrophile groups, the lipophile group having at least eight carbon atoms and the hydrophile group comprising a radical selected from the class consisting of oxygenated sulphur and oxygenated phosphorus inorganic acid radicals, and subjecting the ore pulp to froth flotation.

group comprising a radical selected from the class consisting of oxygenated sulphur and oxygenated phosphorus inorganic acid radicals, and subjecting the ore pulp to froth flotation.

7. In a process for concentrating non-sulfide minerals by flotation, the steps of acidifying pulp to the equivalent of at least 0.1 lb. of sulfuric acid per ton, adding oleic acid and an organic chemical substance having balanced lipophile and hydrophile groups, having at least eight carbon atoms in the lipophile group and the hydrophile group comprising a radical selected from the class consisting of oxygenated sulphur and oxygenated phosphorus inorganic acid radicals, and subjecting the ore pulp to froth flotation.

8. In a process for concentrating non-sulfide minerals by flotation, the steps of acidifying pulp to the equivalent of at least 0.1 lb. of sulfuric acid per ton, adding oleic acid and a sulfuric acid ester of a higher molecular weight aliphatic alcohol, and subjecting the ore pulp to froth flotation, said ester having balanced lipophile and hydrophile groups.

9. In a froth flotation process for concentrating non-sulfide minerals, the step of treating a mass of pulp with an acid to produce a concentration equivalent to at least 0.1 lb. of sulfuric acid per ton of pulp, and adding to the pulp a proportion of free fatty acid and an organic substance having lipophile and hydrophile groups in a state of balance in the molecule, the lipophile group having at least eight carbon atoms and the hydrophile group comprising a radical selected from the class consisting of oxygenated sulphur and oxygenated phosphorus inorganic acid radicals.

10. In a froth flotation process for concentrating non-sulfide minerals, the step of treating a mass of pulp with an acid to produce a concentration equivalent to at least 0.1 lb. of sulfuric acid per ton of pulp, and adding to the pulp a proportion of oleic acid and an organic substance having lipophile and hydrophile groups in a state of balance in the molecule, the lipophile group having at least eight carbon atoms and the hydrophile group comprising a radical selected from the class consisting of oxygenated sulphur and oxygenated phosphorus inorganic acid radicals.

11. A method of concentrating non-sulfide minerals by froth flotation, which comprises treating a mass of pulp with an inorganic acid to produce a relatively strong concentration of acid, adding to the pulp an organic substance having lipophile and hydrophile groups in a state of balance in the molecule, the lipophile group containing at least eight carbon atoms and the hydrophile group comprising a member selected from the class consisting of oxygenated sulphur and oxygenated phosphorus inorganic acid radicals, and a relatively small amount of oleic acid, and subjecting the pulp to froth flotation.

12. A method of concentrating non-sulfide minerals by froth flotation, which comprises forming a pulp of an ore, incorporating with the pulp a proportion of a frother in the form of a relatively high molecular weight fatty acid ester of a polyhydroxy substance wherein one of the hydroxy groups of the polyhydroxy substance is replaced by an oxygenated inorganic acid radical, together with a relatively small amount of a fatty acid as a collector, and subjecting the pulp to froth flotation.

13. In a process for concentrating non-sulfide minerals by flotation, the steps of acidifying pulp to the equivalent of at least 0.1 lb. of sulfuric acid per ton, adding oleic acid and an organic chemical substance having balanced lipophile and hydrophile groups, the lipophile group having at least eight carbon atoms and the hydrophile group comprising a radical selected from the class consisting of oxygenated sulphur and oxygenated phosphorus inorganic acid radicals, and subjecting the ore pulp to froth flotation.

acid per ton, adding oleic acid and a sulphuric acid ester of a polyhydroxy substance partially esterified with a fatty acid, and subjecting the ore pulp to froth flotation.

5 14. A method of concentrating non-sulfide minerals by froth flotation, which comprises forming a pulp of an ore, incorporating with the pulp a proportion of a frother in the form of a relatively high molecular weight fatty acid ester 10 of a polyhydroxy substance wherein one of the hydroxy groups of the polyhydroxy substance is replaced by a sulphonate acid radical, together with a relatively small amount of a fatty acid as a collector, and subjecting the pulp to froth 15 flotation.

15. A method of concentrating non-sulfide minerals by froth flotation, which comprises forming a pulp of an ore, incorporating with the pulp a proportion of monostearine-sulphoacetate 20 and a relatively small proportion of a fatty acid as a collector, and subjecting the pulp to froth flotation.

16. In a process for concentrating non-sulfide materials by froth flotation, the step of adding 25 to an ore pulp a proportion of a chemical substance in the form of a relatively high molecular weight carboxylic acid ester of a polyhydroxy substance wherein at least one hydroxy group of the polyhydroxy substance is esterified with an 30 oxygenated inorganic acid radical.

17. In a process for concentrating non-sulfide materials by froth flotation, the step of adding to an ore pulp a proportion of a chemical substance in the form of a relatively high molecular 35 weight carboxylic acid ester of a polyhydroxy alcohol wherein at least one hydroxy group of the polyhydroxy alcohol is esterified with an oxygenated inorganic acid radical.

18. In a process for concentrating minerals, 40 the step of adding to an ore pulp a proportion of a relatively high molecular weight carboxylic acid ester of a polyhydric alcohol wherein one hydroxy group of the polyhydric alcohol is esterified with a sulphuric acid radical.

45 19. In a process for concentrating minerals, the step of adding to an ore pulp a proportion of a relatively high molecular weight carboxylic acid ester of a polyhydric alcohol wherein one hydroxy group of the polyhydric alcohol is esterified with a sulphuric acid radical, said sulphuric acid radical being neutralized by an alkaline reacting substance.

20. In a process for concentrating minerals, the step of adding to an ore pulp a proportion of a 55 relatively high molecular weight fatty acid ester of glycol wherein one hydroxy group of the glycol is esterified with sulphuric acid.

21. In a process for concentrating minerals, the step of adding to an ore pulp a proportion of a 60 relatively high molecular weight fatty acid ester of glycol wherein one hydroxy group of the glycol is esterified with a sulpho-fatty acid of relatively low molecular weight.

22. In the froth flotation of ores the step which 65 comprises utilizing as a flotation agent a compound having the following general formula:



wherein R is a radical containing a hydrocarbon 70 chain of at least 8 carbon atoms, X is a sulfuric acid or sulfonic acid group present on the extremity of the radical represented by R, and Y is the radical of a salt-forming compound.

23. In the froth flotation of non-sulfide ores 75 the step which comprises utilizing as a flotation

agent a compound having the following general formula:



wherein R represents the residue of a normal primary alcohol containing at least 8 carbon atoms, X represents a sulfuric acid or sulfonic acid group, and Y represents the radical of a salt-forming compound.

24. A froth flotation process which comprises agitating and aerating an aqueous suspension of non-sulfide ores in the presence of a compound having the following general formula:



wherein R represents the residue of a normal 15 primary alcohol having from 8 to 18 carbon atoms.

25. A froth flotation process which comprises frothing a suspension of ore in the presence of a fatty acid collecting agent and a compound 20 having the following general formula:



wherein R represents a radical containing a hydrocarbon group of at least 8 carbon atoms, X 25 represents a sulfuric acid or sulfonic acid group, and Y represents the residue of a salt-forming compound.

26. A froth flotation process which comprises agitating and aerating an aqueous suspension of 30 non-sulfide ores in the presence of a fatty acid collecting agent and a compound having the following general formula:



wherein R represents the residue of a normal 35 primary alcohol containing from 8 to 18 carbon atoms, and Y represents the residue of a salt-forming compound.

27. In the process of concentrating ores by 40 flotation, the step comprising adding to the aqueous flotation medium a salt of a sulphuric acid ester of an aliphatic alcohol having more than nine carbon atoms.

28. In the process of concentrating ores by 45 flotation, the step comprising adding to the aqueous flotation medium sodium dodecyl sulphate, and subjecting the ore to a flotation separation treatment.

29. In the process of concentrating ores by 50 flotation, the step comprising adding to the aqueous flotation medium a salt of a sulphuric acid ester of an aliphatic alcohol having more than nine carbon atoms, and also adding a known flotation agent, and subjecting the ore to a flotation separation treatment.

30. A froth flotation process which comprises agitating and aerating an aqueous suspension of non-sulfide ores in the presence of a collecting 55 agent and a water-soluble compound having the following general formula:



wherein R represents the residue of a normal primary alcohol containing at least 8 carbon atoms, X represents a sulfuric acid or sulfonic 65 acid group and Y represents the residue of a salt-forming compound.

31. A froth flotation process which comprises agitating and aerating an aqueous suspension of non-sulfide ores in the presence of a collecting 70 agent and a water-soluble compound having the following general formula:



wherein R represents the residue of a normal 75

primary alcohol containing from 8 to 18 carbon atoms, X represents a sulfuric acid or sulfonic acid group and Y represents the residue of a salt-forming compound.

5 32. A froth flotation process which comprises agitating and aerating an aqueous suspension of non-sulfide ores in the presence of a collecting agent and a water-soluble compound having the following general formula:



wherein R represents the residue of a normal primary alcohol containing from 12 to 18 carbon atoms, and Y represents the residue of a salt-forming compound.

15 33. The process defined in claim 32 wherein the collecting agent is oleic acid.

34. A froth flotation process which comprises agitating and aerating an aqueous suspension of non-sulfide ores in the presence of a collecting agent and a water-soluble compound having the following general formula:



25 wherein R represents the residue of a normal primary alcohol containing from 12 to 18 carbon atoms.

35. The process defined in claim 34 wherein the collecting agent is oleic acid.

36. A process of separating ores by froth flotation which includes subjecting a pulp of the ore to froth flotation in the presence of an organic nitrogenous substance having lipophile and hydrophile groups in a state of balance in the molecule, the lipophile group having at least 30 eight carbon atoms.

37. A process of separating ores by froth flotation which includes subjecting a pulp of the ore to froth flotation in the presence of an organic nitrogenous substance having lipophile and hydrophile groups in a state of balance in the molecule, the lipophile group containing a hydrocar-

bon radical having at least twelve carbon atoms.

38. A process of separating ores by froth flotation which includes subjecting a pulp of the ore to froth flotation in the presence of an organic nitrogenous substance having lipophile and hydrophile groups in a state of balance in the molecule, the lipophile group containing a straight chain aliphatic radical having at least twelve carbon atoms.

39. A process of separating ores by froth flotation which includes subjecting a pulp of the ore to froth flotation in the presence of a reagent including an organic nitrogen containing halide having a hydrocarbon group containing at least 10 twelve carbon atoms.

40. A process of separating ore by froth flotation which includes subjecting a pulp of the ore to froth flotation in the presence of a reagent including an aliphatic hydrocarbon derivative of 15 pyridinium bromide.

41. A process of separating ores by froth flotation which includes subjecting a pulp of the ore to froth flotation in the presence of a reagent comprising an aliphatic hydrocarbon derivative of 20 a pyridinium halide.

42. The process of claim 41 wherein the aliphatic hydrocarbon group of the reagent contains at least twelve carbon atoms.

43. A process of separating ores by froth flotation which includes subjecting a pulp of the ore to froth flotation in the presence of a reagent comprising an aliphatic derivative of a halide of 25 a heterocyclic compound.

44. The process of claim 43 wherein the aliphatic hydrocarbon group of the reagent contains 30 at least twelve carbon atoms.

45. In the process of concentrating ores by flotation, the step comprising adding to the flotation medium a sulphuric acid ester of a straight chain aliphatic alcohol containing at least eight 35 carbon atoms.

BENJAMIN R. HARRIS.